# EUROPEAN PATENT SPECIFICATION

(11) **EP 0 748 412 B1**
(45) Date of publication and mention of the grant of the patent: **21.10.1998**
(21) Application number: 95912729.1
(22) Date of filing: 02.03.1995
(51) Int. Cl.: D21C 3/22, D21C 1/06, D21C 11/00

(54) **IMPACT OF TEMPERATURE AND ALKALI CHARGE ON PULP BRIGHTNESS**
AUSWIRKUNG VON TEMPERATUR UND ALKALIBELADUNG AUF DEN ZELLSTOFFWEISSGRAD
INCIDENCE DE LA TEMPERATURE ET DE LA CHARGE EN ALCALIS SUR LA BRILLANCE DE LA PATE A PAPIER

(30) Priority: 04.03.1994 US 206496
(43) Date of publication of application: 18.12.1996
(73) Proprietor: BELOIT TECHNOLOGIES, INC., Wilmington, Delaware 19803 (US)
(72) Inventor: SHIN, Nam, Hee, Dalton, MA 01226 (US)
(74) Representative: Schmitz, Jean-Marie
(86) International application number: US9502719
(87) International publication number: WO9523891

(56) References cited:
- EP-A- 0 135 461
- US-A- 1 687 076
- US-A- 4 578 149
- DATABASE WPI Section Ch, Week 9021, Derwent Publications Ltd., London, GB; Class F09, AN 90-162384 & SU,A,1 498 857 (SIBE CELL CARTON) 7 August 1989

## Description

### BACKGROUND OF THE INVENTION

The present invention relates to a process for delignifying and improving the final brightness of pulp. More particularly, the present invention relates to modifications in both the cooking temperature and white liquor charge for a rapid displacement heating cooking system.

Rapid Displacement Heating ("RDH") is a low energy batch cooking process for producing kraft pulp. Combining the inherent advantages of batch cooking with the energy efficiencies of a continuous digester, RDH reuses the spent black liquors that are displaced from a cooked digester to pretreat the wood chips in a consequent cook. Thus, both the chemicals and the heat in these spent liquors are recycled to a consequent cook. The pretreatment of fresh wood chips in a consequent cook begins with lower temperature liquors (approximately 80 ∼ 130°C), and is followed by high temperature liquors (approximately 130° to 165°C) which heat the digester to the highest possible temperature before raising the temperatures to the final cooking temperature (³170°C) with steam.

SU-A-1 498 857 and US-A-1 687 076 are representative of the addition of white liquor to black liquor during impregnation of wood chips in a batch type cooking process, but do not relate to a RDH process.

US-A-4,578,149 and EP-A-0 135 461 teach the basic principles of typical RDH type cooking systems. Specifically, in US-A-4,578,149 there is disclosed a batch digesting process of the type using rapid displacement heating to produce delignified pulp, wherein spent liquor produced in a digeter as a result of cooking a mass of cellulosic material with cooking liquor is displaced and collected in accumulators as hot black liquor and as warm black liquor so as to conserve and utilize the heat of the spent liquor to preheat another mass of cellulosic material in warm black liquor and hot black liquor displacement type pretreatments with progressivly hotter spent liquors prior to cooking. According to US-A-4,578,149, the cooking temperature of the batch ranges from 165°C to 177°C.

RDH and other alkaline cooking processes produce pulp that is relatively dark in color. Greater contrast is usually needed for the many uses of pulp and paper, so pulp is usually bleached to a high brightness in order to make white pulp for writing and printing papers and paperboard. Pulp color arises from changes in the lignin component of the raw material which occur in the pulping process . Unfortunately, with the use of high cooking temperatures and low black liquor strength in the RDH process, low bleachability problems have occurred following the use of conventional, ECF and TCF bleacning processes. High cooking temperatures and low black liquor strength seem to accelerate condensation reactions, resulting in the condensation of lignin with lignin and other wood extractives. As a result, the bleachability of pulp decreased.

An alternative method is, therefore, needed in the RDH cooking process to eliminate such adverse side reactions and improve pulp bleachability.

The object of the present invention is to improve the prior art pulp bleachability in the RDH process.

To achieve this, the batch digesting process of the invention comprises the features of claim 1.

### SUMMARY OF THE INVENTION

The present invention provides a process for improving pulp brightness. Based on modifications to a batch cooking process utilizing rapid displacement heating, the method of the present invention combines the steps of adding white liquor solution (% active alkalinity (AA) or effective alkalinity (EA)) or NaOH to both the warm fill and initial hot fill stages and cooking wood chips at lower temperatures than previously used in a batch type operation to produce pulp that has improved bleachability. In this regard, a total white liquor charge ranging from 15% AA ∼ 35% AA is distributed over the warm, hot and cooking stages in a predetermined amount. If a cool pad is used in practicing the invention, cool white liquor is also added to the black liquor that is released from the cool liquor accumulator. Essentially, white liquor is added to every stage of the batch cooking process prior to the actual cook.

During the cooking of the chips, white and black liquors are present in the digester. Cooking temperatures are low, ranging from 150° ∼ 167°C. With the combination of a high AA or EA white liquor charge and low cooking temperatures, final brightness of pulp is improved. As a result, pollutants and bleaching chemical usage are decreased in pulp mill operations.

### BRIEF DESCRIPTION OF THE DRAWINGS

FIG. 1 illustrates a schematic view of a digester and its associated equipment used in the current RDH cooking system.

FIGS. 2A, 2B and 2C each illustrate white liquor profiling or the addition of white liquor at various stages of the RDH cooking process. In FIG. 2A, plot A represents the addition of a small amount of white liquor at the beginning of the warm fill mode. Plot B represents the cooking stage and illustrates the presence of white liquor in the digester during the actual cooking of the chips.

FIG. 2B illustrates the continuous addition of white liquor to the black liquor at each stage of the RDH cooking process, beginning with the warm fill and continuing through the end of the hot fill. White liquor, as shown, is also present in the digester during the actual cook.

FIG. 2C illustrates the continuous addition of white liquor at each RDH stage including the addition of white liquor to the washer filtrate from the displacement tank.

FIG. 3 illustrates a Stage 3 RDH system without white liquor addition during the warm and hot fill modes.

FIG. 4 illustrates a Stage 3 RDH system with the addition of white liquor during the warm and hot fill modes.

FIG. 5 illustrates a plot of D1-brightness versus total (D100 + D1) available chlorine charge for the best case and baseline case RDH pulps. Plot A represents RDH pulp R3 (0.225 Kappa factor). Plot B represents RDH pulp R4 (0.27 Kappa factor). Plot C represents RDH pulp R7 (0.225 Kappa factor). Plot D represents RDH pulp R8 (0.27 Kappa factor).

FIG. 5A illustrates a plot of D1-brightness versus D1-chlorine dioxide charge. Plot A represents RDH pulp R3 (0.225 Kappa factor). Plot B represents RDH pulp R4 (0.27 Kappa factor). Plot C represents RDH pulp R7 (0.225 Kappa factor). Plot D represents RDH pulp R8 (0.27 Kappa factor).

FIG. 6 illustrates the D1-brightness versus the total available chlorine charge in the D100- and D1-stages for all 0.225 Kappa factor bleaches. Plot A represents RDH pulp R3. Plot B represents RDH pulp R12. Plot C represents RDH pulp R7.

FIG. 6A illustrates the D1-brightness versus the D1-stage chlorine dioxide charges. Plot A represents RDH pulp R3 (0.225 Kappa factor). Plot B represents RDH pulp R12 (0.225 Kappa factor). Plot C represents RDH pulp R7 (0.225 Kappa factor).

FIG. 7 illustrates the D1-brightness versus the total available chlorine charge in the D100- and D1-stages for all 0.27 Kappa factor bleaches. Plot A represents RDH pulp R4. Plot B represents RDH pulp R12. Plot C represents RDH pulp R8.

FIG. 7A illustrates the D1-brightness versus the D1-stage chlorine dioxide charges. Plot A represents RDH pulp R4 (0.27 Kappa factor). Plot B represents RDH pulp R12 (0.27 Kappa factor). Plot C represents RDH pulp R8 (0.27 Kappa factor).

### DETAILED DESCRIPTION OF THE PRESENTLY PREFERRED EMBODIMENTS

The present invention as described in claim 1 provides a process for improving pulp bleachability, which is based on modifications to the existing RDH Cooking System for the digestion of wood chips. More specifically, the process involves the addition of a white liquor charge commencing at the start of the RDH cooking cycle and continuing until the time to temperature stage of the process, at which time the actual cook begins. The process of the present invention is also predicated on the use of somewhat lower cooking temperatures for the actual cook as compared to cooking temperatures commonly used in the RDH pulping process.

In accordance with the present invention, a total white liquor charge ranging between approximately 15%AA ∼ 35%AA is distributed over the warm black liquor, initial hot black liquor and cooking stages. When used, the cool pad or cool liquor accumulator also receives a white liquor charge. In addition to the use of a distributed white liquor charge, the present invention utilizes lower cooking temperatures ranging between approximately 150°C ∼ 167°C. As a result, pulp is produced which, upon bleaching with any combination of bleaching chemicals, is improved in final brightness.

The operational stages for a typical RDH Cooking System are as follows: (1) chip fill; (2) cool black liquor fill; (3) warm black liquor fill; (4) hot black liquor fill; (5) time to temperature; (6) time at temperature; (7) displacement; and (8) pump out. The basic principles of RDH operation are described in US-A-4,578,149 (issued March 25, 1986). Accordingly, details of RDH operations will be discussed only to the extent necessary for one of ordinary skill in the art to appreciate the modifications in the RDH cooking system, which produce the bleachable grade pulp described herein.

FIG. 1 schematically illustrates the type of apparatus for RDH that is used for the digestion of pulp. It should be understood that this figure illustrates very general features of the cooking apparatus, and modifications and variations in this system are indeed made as will be discussed in greater detail below. Many instrumentalities such as gauges, pressure vents, pumps and valves have been eliminated from the figures disclosed herein for reasons of simplicity. FIG. 1 is used to illustrate the existing RDH cooking process and to facilitate an understanding of the improvements to the process in accordance with the principles of the present invention.

Referring to FIG. 1, a digester is illustrated at 10 of the type generally used in the chemical digestion of wood chips. The digester 10 has a truncated bottom 12. An inlet valve 14 controls the entry of various reactive liquors into digester 10. Although not shown, the contents of digester 10 can be heated to a final cooking temperature by pumping cooking liquor through a heat exchanger or steam sparger which is connected to digester 10 by a valve-controlled line.

After the wood chips are added to digester 10, cool black liquor (temperature around 70°-95°C) from the cool liquor accumulator (A tank) 16 is pumped by means of pump 18 through line 20 which is controlled by a valve 22 into the bottom of the digester 10 through an inlet valve 14. Next, warm black liquor (temperature between approximately 90°-150°C) from the warm liquor accumulator 24 is pumped out by means of a pump 18 through a valve 22 and through valve 14 into the bottom of digester 10. During this warm liquor fill, some black liquor is displaced from the digester 10 and then returned by a line 26 to the cool liquor accumulator 16. Hot black liquor (temperature between 150°-168°C) is then pumped from the hot liquor accumulator (C tank) 28 by means of a pump 30 which is controlled by a valve 32 into the bottom of the digester 10 utilizing valve 14. During the hot fill, black liquor is displaced from the digester 10 and returned to the warm liquor accumulator 24 and hot liquor accumulator 28 through lines 34 and 36, respectively. During the middle of the hot fill, hot white liquor stored in the hot white liquor accumulator 38 is pumped out by means of a pump 30 where it combines with the hot black liquor leaving the hot liquor accumulator 28, the combined liquors then passing through a valve 32 and into the base of the digester 10.

After the hot fill is completed, the inlet and outlet valves to the digester 10 are closed as the time to temperature stage commences. Steam is injected into the digester 10 and the temperature is increased to the cooking temperature, which averages approximately 170°C. The temperature of the digester is maintained at about this temperature until the wood chips are digested, depending on white liquor charge and H-factor.

Upon completion of the cooking stage, washer filtrate (temperature approximately 70 ∼ 85°C) stored in a displacement tank (D tank) 40 is pumped into the digester 10, utilizing pump 42 and valve 44. The contents are washed and the digester 10 is cooled. As the washer filtrate is added to the digester 10, the spent liquors are displaced and returned to the warm liquor accumulator 24 and the hot liquor accumulator 28 by lines 46 and 48, respectively. The displacement mode is concluded when all washer filtrate is used, which is based on the dilution factor of the washer. After displacement is completed, the digested pulp is then pumped out of the digester 10 to a discharge tank using pump 50.

With the current RDH cooking system, cooking temperatures of greater than 170°C are used for rapid cooking, resulting in the acceleration of condensation reactions. As a result, bleachability problems occurred when the pulp was subjected to conventional, ECF and TCF bleaching processes. The present invention overcomes these problems and improves pulp bleachability by modifying the cooking process for wood chips. This improved RDH process utilizes a combination of higher alkalinity (or white liquor charge) and lower cooking temperatures. More specifically, white liquor is added during the warm and initial hot fill stages. This is in contrast to the existing RDH cooking process, wherein white liquor is added only during the middle of the hot fill mode. Further, when a cool pad is used in the present invention, white liquor is added to the cool black liquor leaving the cool liquor accumulator (or A tank). Thus, from the beginning of the RDH cooking process until the time to temperature stage, white liquor is added during each stage to the black liquor. The addition of white liquor at every stage, also called white liquor profiling, is illustrated in greater detail below in FIGS. 2A, 2B and 2C.

In FIG. 2A, plot A illustrates the addition of a small amount of white liquor at the beginning of the warm fill mode when warm black liquor leaves the B tank or warm liquor accumulator and flows to the digester. White liquor can also be added to the A tank or cool pad when used. At the end of the hot fill mode, which utilizes two hot liquor accumulators C1 and C2, the mixture of white and black liquors remains in the digester. Plot B represents the cooking stage and illustrates the presence of white liquor in the digester during the actual cooking of the chips. Black liquor is also present during the cook.

FIG. 2B illustrates the continuous addition of white liquor to black liquor at each stage of the cooking process, beginning with the warm fill through the end of the hot fill mode.

FIG. 2C illustrates the continuous addition of white liquor throughout the various stages, including the addition of white liquor to the washer filtrate from the displacement tank.

The concentration of dissolved organic material in the initial hot fill operation (C1 and C2 tanks containing black liquor) was compared with and without white liquor addition during the warm and hot fill operations. FIG. 3 illustrates a Stage 3 RDH system where no white liquor is added during the warm and hot fill modes. Only warm black liquor is leaving the warm liquor accumulator (B tank) 24 to flow through line 56 during the warm fill mode and into line 20, which then empties into the digester 10. Although this RDH system contains two hot liquor accumulators 28 (C1 tank) and 58 (C2 tank), respectively, there are RDH pulping processes which utilize only one hot liquor accumulator. In practicing the present invention, it is contemplated that the process of white liquor profiling can be applied to systems having any number of black liquor accumulators.

As shown in FIG. 3, during the initial hot fill mode, hot black liquor leaves the hot liquor accumulators 28 and 58 by lines 60 and 62, respectively, and flows to the digester 10 through lines 64 and 20. During the middle of the hot fill, hot white liquor from the hot white liquor accumulator 38 mixes with the hot black liquor leaving hot liquor accumulator 58 by line 66. The mixture then flows through lines 64 and 20 and into the digester 10.

FIG. 4 illustrates a Stage 3 RDH System with the addition of white liquor during the warm and hot fill modes. First, during the warm fill, white liquor is added to the warm black liquor leaving the warm liquor accumulator 24 by line 70. The warm fill flows through lines 56 and 20 into the digester 10. Either cool or hot white liquor may be used during the warm fill mode. During the initial hot fill mode, hot white liquor from the hot white liquor accumulator 38 is mixed with black liquor leaving hot liquor accumulator 28 by line 72, and is further mixed with the black liquor exiting 'the second hot liquor accumulator 58 by lines 62 and 66. The mixture of hot white and black liquors flows from the two hot liquor accumulators 28 and 58 through lines 64 and 20 into the digester 10.

The results of the comparison are as follows:

| *Without White Liquor Addition* at Warm and Hot Fill Operations (FIG. 3) | | |
|---|---|---|
| Initial Hot Fill Operation | Total Flow. gal*/cook | Dissolved Organic. % |
| C1 black liquor | 20799 | 13.1 |
| C2 black liquor | 8709 | 14.9 |

| | | |
|---|---|---|
| * 1 gallon = 3,785 l | | |

*With White Liquor Addition* at Warm and Hot Fill Operations (FIG. 4)
- White Liquor charges:: 1.5% AA at C1 black liquor
1.5% AA at C2 black liquor

| Initial Hot Fill Operation | Total Flow. gal*/cook | Dissolved Organic. % |
|---|---|---|
| C1 Black liquor | 19877 | 10.1 |
| C2 black liquor | 7971 | 9.8 |

| | | |
|---|---|---|
| * 1 gallon = 3,785 l | | |

This case study clearly demonstrates that the concentration of dissolved organic compounds at initial hot fill operation can be adjusted by adding white liquor to the hot fill line. The concentration of dissolved organic compounds in the C1 black liquor and in the C2 black liquor decreases from 13.1% to 10.1% and 14.9% to 9.8%, respectively.

In order to maximize bleachability benefits and extend delignification for the RDH process, warm black liquor (temperatures between approximately 70° and 150°C and its strength between 3 and 20 g/l AA) and hot black liquor (temperatures between approximately 100° and 168°C and its strength between 8 and 30 g/l AA) should be reinforced with any combination of white liquor or NaOH solution.

As shown in the figures presented above, warm and hot black liquor can be modified using white liquor profiling. These liquors can also be modified by sodium hydroxide (NaOH) profiling. The addition of white liquor or NaOH controls the total dissolved solids (TDS) concentration and black liquor strength using any combination of black liquor, white liquor and NaOH. The washer filtrate displacement stage, in which the black liquor temperature is held between approximately 50° and 105°C and black liquor strength between 1 and 18 g/l AA, can be reinforced with any combination of white liquor or NaOH solution.

By way of example, and not limitation, the following examples serve to further illustrate the present invention in its preferred embodiments.

As shown below, Tables 1, 1A, 2, 2A, 3 and 3A provide the pulping results and conditions for a number of cooks used in preparing the RDH pulps for subsequent bleaching studies. A summary of the pulping results is provided in Table 3B.

**TABLE 1**

| RDH Pulping Conditions and Results - "Best Case" | | | | | | | | |
|---|---|---|---|---|---|---|---|---|
| Cook Number | R1 | Post R1 | R2 | Post R2 | R3 | Post R3 | R4 | Post R4 |
| H factor | 937 | | 532 | | 475 | | 452 | |
| AA (TAPPI) to Hot Fill, % | 16.0 | | 16.0 | | 16.0 | | 16 | |
| Sulfidity (TAPPI), on AA | 30.4 | | 30 | | 30.3 | | 30. 2 | |
| Maximum temp, C | 160 | | 160 | | 160 | | 160 | |
| Time to max, min | 16 | | 20 | | 17 | | 19 | |
| Time at max, min | 130 | | 37 | | 60 | | 57 | |
| Kappa, unscreened | 7.2 | | 8.9 | | 9.2 | | 9.8 | |
| Kappa, screened | 7.1 | | 8.2 | | 8.8 | | 9.3 | |
| Total yield, % | 46.3 | | 47.3 | | 48.2 | | 1.7 | |
| Total rejects,% | 0.9 | | 1.2 | | 1.4 | | 1.7 | |
| Screened yield,% | 45.4 | | 46.1 | | 46.8 | | 46. 9 | |
| Viscosity,0 .5k CED, cp | 26 | | 39 | | 40.7 | | 44. 9 | |
| | | | | | | | | |

| **End of Cook Residual:** | | | | | | | | |
|---|---|---|---|---|---|---|---|---|
| AA(Na2O), g/L | 28.2 | | 31.6 | | 32.9 | | 31. 6 | |
| EA (Na20), g/L | 21.1 | | 24.2 | | 24.2 | | 24. 2 | |
| Na2S (Na20), g/L | 14.3 | | 14.9 | | 17.4 | | 14. 9 | |
| TTA(Na2O),g /L | | | | | | | | |
| Solids,% | 14.8 | | 15.9 | | 16.7 | | 16. 8 | |
| Solids.g/L | 161 | | 173 | | 183 | | 185 | |
| Sulfidity % on A.A. | 51 | | 47.1 | | 52.9 | | 47. 1 | |

| **HOT FILL:** | | | | | | | | |
|---|---|---|---|---|---|---|---|---|
| Hot liquor charge, L | 18 | | 18 | | 18 | | 18 | |
| Charge time, min | 13 | | 14 | | 13 | | 13 | |
| Temperature , C | | | | | | | | |
| Top | 130 | | 127 | | 127 | | 128 | |
| Bottom | 145 | | 141 | | 141 | | 141 | |

| **Chemical Conditions in Accumulator:** | | | | | | | | |
|---|---|---|---|---|---|---|---|---|
| AA(Na2O), g/L | 22.9 | 20.6 | 25.7 | 21.7 | 29.2 | 24.6 | 27. 3 | 23.6 |
| EA (Na20), g/L | 16.1 | 15.1 | 18.1 | 16.1 | 20.2 | 18.3 | 19. 8 | 17.9 |
| Na2S (Na20), g/L | 13.7 | 11 | 15.2 | 11.2 | 18 | 12.7 | 14. 9 | 11.4 |
| TTA (Na20), g/L | - | - | - | - | - | - | - | - |
| Sulfidity, % on A.A. | 59.4 | 53.4 | 59.1 | 51.6 | 61.6 | 51.2 | 54. 9 | 48.3 |
| Solids,% | 9.5 | 10.5 | 11.1 | 11.9 | 11.9 | 13.6 | 12. 7 | 13.6 |
| Solids, g/L | 99.8 | 111 | 118 | 127 | 127 | 146 | 137 | 146 |
| Total elapsed time, min* | 45 | | 43 | | 41 | | 42 | |

| | | | | | | | | |
|---|---|---|---|---|---|---|---|---|
| * includes heating time to 145°C and time at 145°C after initial hot black liquor injection and final hot BIL with WIL mix. | | | | | | | | |

**TABLE 1A**

| RDH Pulping Conditions and Results "Best Case" | | | | | | | | |
|---|---|---|---|---|---|---|---|---|
| Cook Number | R1 | Post R1 | R2 | Post R2 | R3 | Post R3 | R4 | Post R4 |

| WHITE LIQUOR | | | | | | | | |
|---|---|---|---|---|---|---|---|---|
| White liquor charge,L | 6.04 | | 5.65 | | 5.53 | | 5.52 | |
| Hot B/L,L | 5 | | 4.13 | | 5.5 | | 5.8 | |
| Charge time, min | 11 | | 11 | | 9 | | 9 | |
| Temperature, C | | | | | | | | |
| Top | 140 | | 139 | | 140 | | 139 | |
| Bottom | 141 | | 141 | | 144 | | 143 | |

| **Chemical conditions in accumulator: (TAPPI)** | | | | | | | | |
|---|---|---|---|---|---|---|---|---|
| AA (Na2o), g/L | 98 | | 99.2 | | 10.2 | | 101.5 | |
| EA(Na2O) g/L | 83.1 | | 84.3 | | 85.8 | | 86.2 | |
| Na2S (Na2O), g/L | - | | - | | - | | - | |
| TTA (Na20), g/L | | | | | | | | |
| Sulfidity, %on AA | 30.4 | | 30 | | 30.3 | | 30.2 | |

| **CHIP CHARGE & LIQUOR PACKING:** | | | | | | | | |
|---|---|---|---|---|---|---|---|---|
| Chip charge, g | 3,700 | | 3,500 | | 3,50 0 | | 3,50 0 | |
| Chip Moisture, % | 37.3 | | 37.3 | | 37.3 | | 37.3 | |
| O.D. Solids, % | 62.7 | | 62.7 | | 62.7 | | 62.7 | |

| **WARM FILL:** | | | | | | | | |
|---|---|---|---|---|---|---|---|---|
| Warm Liquor charge, L | 24.7 | | 24 | | 24 | | 24 | |
| Exit pH, initial | 12.8 | | 13.5 | | 13.3 | | 13.3 | |
| Charge time, min | 15 | | 15 | | 15 | | 15 | |
| Temperature, C | | | | | | | | |
| Top | 100 | | 104 | | 102 | | 100 | |
| Bottom | 113 | | 112 | | 111 | | 112 | |

| **Chemical conditions in Accumulator:** | | | | | | | | |
|---|---|---|---|---|---|---|---|---|
| AA(Na2O), g/L | 23.6 | 16.4 | 26.4 | 17.7 | 25.7 | 19.2 | 28.5 | 21.1 |
| EA (Na2O), g/L | 16.4 | 10.5 | 17.4 | 11.5 | 18 | 12.4 | 18.6 | 13.6 |
| Na2S (Na2O), g/L | 14.3 | 11.8 | 18 | 12.4 | 15.5 | 13.6 | 19.8 | 14.9 |
| TTA (Na2O), g/L | - | - | - | - | - | - | - | - |
| Sulfidity, % on A.A. | 60.8 | 71.7 | 68.3 | 70.2 | 60.3 | 71 | 69.5 | 70.6 |
| Solids, % | 9 | 9.25 | 13.6 | 12.4 | 14.3 | 13.1 | 14.1 | 13.1 |
| Solids, g/L | 94.3 | 96.4 | 147 | 131 | 155 | 141 | 152 | 141 |
| Total elapsed time, min* | 40 | | 31 | | 34 | | 33 | |

| **DISPLACEMENT**: | | | | | | | | |
|---|---|---|---|---|---|---|---|---|
| Displaceme nt Volume, L | 32 | | 32 | | 32 | | 32 | |
| Charge time, min | 26 | | 26 | | 26 | | 26 | |

| **Chemical Conditions in accumulator: (TAPPI)** | | | | | | | | |
|---|---|---|---|---|---|---|---|---|
| AA (Na2O), g/L | 9.5 | | 10.1 | | 9 | | 10.1 | |
| EA (Na2O), g/L | 9.5 | | 10.1 | | 9 | | 10.1 | |
| Na2S (Na2O), g/L | - | | - | | - | | - | |
| TTA (Na2O), g/L | - | | - | | - | | - | |
| Sulfidity, % on A.A. | 0 | | 0 | | 0 | | 0 | |

| | | | | | | | | |
|---|---|---|---|---|---|---|---|---|
| * includes fill time, heating time to 120°C and time at 120°C after warm fill. | | | | | | | | |

**TABLE 2**

| RDH Pulping Conditions and Results - "Baseline Case" | | | | | | | | |
|---|---|---|---|---|---|---|---|---|
| Cook Number | R5 | Post R5 | R6 | Post R6 | R7 | Post R7 | R8 | Post R8 |
| H factor | 1161 | | 765 | | 831 | | 832 | |
| AA (TAPPI) to Hot Fill, % | 10.0 | | 10.0 | | 10.0 | | 10.0 | |
| Sulfidity (TAPPI),% on AA | 30. 2 | | 30.3 | | 30.3 | | 30.2 | |
| Maximum temp, C | 170 | | 170 | | 170 | | 170 | |
| Time to max, min | 23 | | 27 | | 21 | | 21 | |
| Time at max, min | 62 | | 35 | | 41 | | 42 | |
| Kappa, unscreene d | 7.6 | | 9.7 | | 9.5 | | 8.9 | |
| Kappa, screened | 7.2 | | 9.1 | | 8.9 | | 8.8 | |
| Total yield,% | 47.3 | | 48.3 | | 48.6 | | 49.1 | |
| Total rejects,% | 1.1 | | 1.6 | | 1.7 | | 1.4 | |
| Screened yield,% | 46.2 | | 46.7 | | 46.9 | | 47.7 | |
| Viscosity, 0.5% CED, cp | 19.5 | | 33.2 | | 33.3 | | 32.2 | |
| | | | | | | | | |

| **End of Cook Residual:** | | | | | | | | |
|---|---|---|---|---|---|---|---|---|
| AA(Na2O) , g/L | 27.9 | | 25.4 | | 26 | | 25.4 | |
| EA (Na2O), g/L | 19.2 | | 18 | | 17.4 | | 17.4 | |
| Na2S (Na2O), g/L | 17.4 | | 14.9 | | 17.4 | | 16 | |
| TTA(Na2O) , g/L | | | | | | | | |
| Solids,% | 19 | | 19.1 | | 19.2 | | 19.1 | |
| Solids,g/L | 210 | | 211 | | 213 | | 210 | |
| Sulfidity % on A.A. | 62.4 | | 58.3 | | 66.2 | | 63 | |

| **HOT FILL:** | | | | | | | | |
|---|---|---|---|---|---|---|---|---|
| Hot liquor charge, L | 18 | | 18 | | 18 | | 18 | |
| Charge time, min | 12 | | 13 | | 12 | | 13 | |
| Temperatu re, C | | | | | | | | |
| Top | 135 | | 137 | | 137 | | 135 | |
| Bottom | 153 | | 153 | | 154 | | 155 | |

| **Chemical conditions in Accumulator:** | | | | | | | | |
|---|---|---|---|---|---|---|---|---|
| AA(Na2O) , g/L | 30.4 | 23.6 | 26 | 21.1 | 26.7 | 20.5 | 26.4 | 20.5 |
| EA (Na2O), g/L | 22.3 | 16.2 | 18.6 | 14.3 | 18 | 13.6 | 18.3 | 13.6 |
| Na2S (Na2O), g/L | 16.1 | 14.9 | 14.9 | 13.6 | 17.4 | 13.6 | 16.1 | 13.6 |
| TTA (Na2O), g/L | - | - | - | - | - | - | - | - |
| Sulfidity, % on A.A. | 53. 3 | 63.6 | 56.9 | 64.5 | 65.2 | 67.3 | 61.4 | 67.3 |
| Solids,% | 16. 7 | 17 | 17.2 | 17.1 | 17 | 17.3 | 17 | 16.9 |
| Solids, g/L | 183 | 185 | 189 | 187 | 187 | 189 | 186 | 184 |
| Total elapsed time, min* | 46 | | 44 | | 45 | | 44 | |

| | | | | | | | | |
|---|---|---|---|---|---|---|---|---|
| * includes heating time to 155°C and time at 155°C after initial hot black liquor injection and final hot B/L with W/L mix. | | | | | | | | |

**TABLE 2A**

| RDH Pulping Conditions and Results - "Baseline Case" | | | | | | | | |
|---|---|---|---|---|---|---|---|---|
| Cook Number | R5 | Post R5 | R6 | Post R6 | R7 | Post R7 | R8 | Post R8 |

| **WRITE LIQUOR:** | | | | | | | | |
|---|---|---|---|---|---|---|---|---|
| White liquor charge,L | 3.47 | | 3.45 | | 3.46 | | 3.47 | |
| Hot B/L,L | 5.4 | | 7 | | 5.6 | | 5 | |
| Charge time, min | 9 | | 9 | | 9 | | 9 | |
| Temperature, C | | | | | | | | |
| Top | 151 | | 152 | | 151 | | 151 | |
| Bottom | 149 | | 147 | | 145 | | 144 | |

| **chemical conditions in accumulator; (TAPPI)** | | | | | | | | |
|---|---|---|---|---|---|---|---|---|
| AA (Na2O), g/L | 100.8 | | 101.4 | | 101.2 | | 100. 8 | |
| EA(Na2O) g/L | 85.6 | | 86 | | 85.9 | | 85.6 | |
| Na2S (Na2O), g/L | - | | - | | - | | - | |
| TTA (Na2O), g/L | 121.6 | | 122.8 | | 123.1 | | 120. 6 | |
| Sulfidit y, % on AA | 30.2 | | 30.3 | | 30.3 | | 30.2 | |

| **CHIP CHARGE & LIQUOR PACKING:** | | | | | | | | |
|---|---|---|---|---|---|---|---|---|
| Chip charge, g | 3,500 | | 3,500 | | 3,500 | | 3,50 0 | |
| Chip Moisture , % | 37.3 | | 37.3 | | 37.3 | | 37.3 | |
| O.D. Solids, % | 62.7 | | 62.7 | | 62.7 | | 62.7 | |

| WARM FILL: | | | | | | | | |
|---|---|---|---|---|---|---|---|---|
| Warm Liquor charge, L | 24.4 | | 25 | | 25.2 | | 24 | |
| Exit pH, initial | 13.1 | | 13.3 | | 13.5 | | 13.3 | |
| Charge time, min | 15 | | 15 | | 15 | | 15 | |
| Temper-a ture, C | | | | | | | | |
| Top | 109 | | 109 | | 106 | | 106 | |
| Bottom | 121 | | 120 | | 118 | | 116 | |

| **Chemical conditions in Accumulator: (TAPPI)** | | | | | | | | |
|---|---|---|---|---|---|---|---|---|
| AA(Na2O) g/L | 28.1 | 19.2 | 27.9 | 18.6 | 26.7 | 19.2 | 26.7 | 19.7 |
| EA (Na2O), g/L | 18.3 | 12.4 | 18 | 11.2 | 18 | 11.8 | 18.6 | 12.1 |
| Na2S (Na2O), g/L | 19.6 | 13.6 | 19.8 | 14.9 | 17.4 | 14.9 | 16.1 | 15.1 |
| Sulfidit y, % on A.A. | 69.8 | 70.8 | 71 | 79.6 | 65.2 | 77.1 | 60.7 | 77.2 |
| Solids, | 14.5 | 15.4 | 15 | 16 | 14.7 | 15.5 | 14.6 | 15.9 |
| Solids, g/L | 157 | 167 | 164 | 173 | 159 | 168 | 158 | 172 |
| Total elapsed time, min* | 35 | | 33 | | 31 | | 30 | |

| **DISPLACEMENT:** | | | | | | | | |
|---|---|---|---|---|---|---|---|---|
| Displace -ment Volume, L | 32 | | 32 | | 32 | | 32 | |
| Charge time, min | 26 | | 26 | | 26 | | 26 | |

| **Chemical Conditions in accumulator:** | | | | | | | | |
|---|---|---|---|---|---|---|---|---|
| AA (Na2O), g/L | 4.3 | | 4.31 | | 4.3 | | 4.3 | |
| EA (Na2O), g/L | 3.7 | | 3.7 | | 3.7 | | 3.5 | |
| Na2S (Na2O), g/L | 1.24 | | 1.24 | | 1.24 | | 1.74 | |
| Sulfidit y, % on A.A. | 27.9 | | 27.9 | | 27.9 | | 27.9 | |
| Solids, % | 9.7 | | 10.6 | | 10.4 | | 10.3 | |
| Solids, g/L | 102 | | 112 | | 109 | | 108 | |

| | | | | | | | | |
|---|---|---|---|---|---|---|---|---|
| * includes fill time, heating time to 120°C and time at 120°C after warm fill. | | | | | | | | |

**TABLE 3**

| **RDH Pulping Conditions and Results -"Best Do-able Case"** | | | | | | | | |
|---|---|---|---|---|---|---|---|---|
| Cook Number | R9 | Post R9 | R10 | Post R10 | R11 | Post R11 | R12 | Post R12 |
| H factor | 484 | | 558 | | 483 | | 494 | |
| AA(TAPPI) to Hot Fill, % | 18.9 | | 16.0 | | 16.0 | | 16 | |
| Sulfidity (TAPPI),% on AA | 30.6 | | 30.2 | | 29.8 | | 30.4 | |
| Maximum temp, C | 160 | | 160 | | 160 | | 160 | |
| Time to max, min | 20 | | 20 | | 18 | | 16 | |
| Time at max, min | 60 | | 72 | | 62 | | 63 | |
| Kappa, unscreened | 9.1 | | 8.9 | | 9.6 | | 10 | |
| Kappa, screened | 8.1 | | 8.5 | | 9.2 | | 9.3 | |
| Total yield,% | 48.1 | | 48.1 | | 49.1 | | 49.1 | |
| Total rejects,% | 1.1 | | 1.2 | | 1.5 | | 1.3 | |
| Screened yield,% | 47 | | 46.9 | | 47.6 | | 47.8 | |
| Viscosity,0.5% CED, cp | 33.5 | | 33 | | 39.3 | | 32.1 | |

| **End of Cook Residual:** | | | | | | | | |
|---|---|---|---|---|---|---|---|---|
| AA(Na2O), g/L | 37.6 | | 32.8 | | 34.1 | | 33.5 | |
| EA (Na2O), g/L | 28.6 | | 25.3 | | 25.9 | | 25.3 | |
| Na2S (Na2O), g/L | 17.9 | | 15.2 | | 16.4 | | 16.4 | |
| Solids,% | 18.8 | | 19.1 | | 19.2 | | 19.3 | |
| Solids, g/L | 210 | | 212 | | 215 | | 214 | |
| Sulfidity % on A.A. | 47.9 | | 45.7 | | 48.1 | | 49 | |

| **HOT FILL:** | | | | | | | | |
|---|---|---|---|---|---|---|---|---|
| Hot liquor charge, L | 18 | | 18 | | 18 | | 18.7 | |
| Charge time, min | 13 | | 13 | | 13 | | 13 | |
| Temperature , C | | | | | | | | |
| Top | 129 | | 132 | | 132 | | 132 | |
| Bottom | 145 | | 147 | | 147 | | 145 | |

| **Chemical conditions in Accumulator:** | | | | | | | | |
|---|---|---|---|---|---|---|---|---|
| AA(Na2O), g/L | 27.8 | 25.9 | 27.3 | 25.3 | 27.1 | 24.6 | 26.5 | 23.4 |
| EA (Na2O), g/L | 19.9 | 18.9 | 19.9 | 18.3 | 20.2 | 18.3 | 19.5 7 | 17 |
| Na2S (Na2O), g/L | 15.8 | 13.4 | 14.9 | 13.9 | 13.9 | 12.6 | 13.9 | 12.6 |
| TTA (Na2O), g/L | - | - | - | - | - | - | - | - |
| Sulfidity, % on A.A. | 56.8 | 54.1 | 54.2 | 55.3 | 50.9 | 51.2 | 52.3 | 54.7 |
| Solids,% | 16.2 | 16.1 | 16.7 | 16.7 | 17 | 17.2 | 17.3 | 17 |
| Solids, g/L | 177 | 176 | 182 | 183 | 187 | 189 | 190 | 186 |
| Total elapsed time, min* | 42 | | 42 | | 42 | | 39 | |

| | | | | | | | | |
|---|---|---|---|---|---|---|---|---|
| * includes heating time to 145°C and time at 145°C after initial hot black liquor injection and final hot B/L with W/L mix. | | | | | | | | |

**TABLE 3A**

| RDH Pulping Conditions and Results - "Best Do-able Case" | | | | | | | | |
|---|---|---|---|---|---|---|---|---|
| Cook Number | R9 | Post R9 | R10 | Post R10 | R11 | Post R11 | R12 | Post R12 |

| **WHITE LIQUOR:** | | | | | | | | |
|---|---|---|---|---|---|---|---|---|
| White liquor charge,L | 6.17 | | 5.81 | | 5.79 | | 5.6 | |
| Hot B/L,L | 4.8 | | 5.2 | | 5.0 | | 6.4 | |
| Charge time, min | 10 | | 10 | | 10 | | 9 | |
| Temperature, C | | | | | | | | |
| Top | 139 | | 140 | | 139 | | 141 | |
| Bottom | 139 | | 145 | | 140 | | 144 | |

| **Chemical conditions in accumulator: (TAPPI)** | | | | | | | | |
|---|---|---|---|---|---|---|---|---|
| AA (Na2O), g/L | 107.3 | | 96.4 | | 96.7 | | 100 | |
| EA(Na2O) g/L | 90.8 | | 81.8 | | 82.3 | | 84.8 | |
| TTA (Na2O), g/L | 125.8 | | 115.6 | | 117.8 | | 120.9 | |
| Sulfidit y, % on AA | 30.6 | | 30.2 | | 29.8 | | 30.4 | |

| **CHIP CHARGE & LIQUOR PACKING:** | | | | | | | | |
|---|---|---|---|---|---|---|---|---|
| Chip charge, g | 3,500 | | 3,500 | | 3,500 | | 3,50 0 | |
| Chip Moisture , % | 37.3 | | 37.3 | | 37.3 | | 37.3 | |
| O.D. Solids, | 62.7 | | 62.7 | | 62.7 | | 62.7 | |

| **WARM FILL:** | | | | | | | | |
|---|---|---|---|---|---|---|---|---|
| Warm Liquor charge, L | 24.5 | | 24.3 | | 23.9 | | 24.2 | |
| Exit pH, initial | 13.3 | | 13.2 | | 13.2 | | 13 | |
| Charge time, min | 15 | | 15 | | 15 | | 15 | |
| Temperature, C | | | | | | | | |
| Top | 108 | | 106 | | 104 | | 108 | |
| Bottom | 121 | | 117 | | 116 | | 118 | |

| **Chemical conditions in Accumulator: (TAPPI)** | | | | | | | | |
|---|---|---|---|---|---|---|---|---|
| AA(Na2O) , g/L | 27.1 | 21.1 | 26.5 | 21.1 | 26.5 | 20.8 | 25.9 | 20.8 |
| EA (Na2O), g/L | 20.5 | 14.5 | 18.9 | 14.1 | 18.3 | 13.3 | 17.7 | 13.3 |
| Na2S (Na2O), g/L | 13.3 | 13.3 | 15.2 | 14.1 | 16.4 | 15.2 | 16.4 | 15.2 |
| Sulfidit y, % on A.A. | 48.7 | 62.6 | 57.4 | 66.4 | 61.9 | 72.1 | 63.3 | 72.1 |
| Solids, % | 14.3 | 14.9 | 14.8 | 15.8 | 15.6 | 16.1 | 15 | 15.6 |
| Solids, g/L | 155 | 161 | 162 | 171 | 170 | 176 | 163 | 170 |
| Total elapsed time, min* | 30 | | 30 | | 31 | | 30 | |

| **DISPLACEMENT:** | | | | | | | | |
|---|---|---|---|---|---|---|---|---|
| Displace -ment Volume, L | 32 | | 32 | | 32 | | 32 | |
| Charge time, min | 26 | | 26 | | 26 | | 26 | |
| | | | | | | | | |

| **Chemical Conditions in accumulator: (TAPPI)** | | | | | | | | |
|---|---|---|---|---|---|---|---|---|
| AA (Na2O), g/L | 9.5 | | 9.8 | | 8.8 | | 11.4 | |
| EA (Na2O), g/L | 8.2 | | 9.2 | | 8.2 | | 10.7 | |
| Na2S (Na2O), g/L | 2.5 | | 1.3 | | 1.3 | | 1.3 | |
| Sulfidit y, % on A.A. | 31.7 | | 13 | | 14.6 | | 13.1 | |
| Solids, | 10.3 | | 10.6 | | 11.2 | | - | |
| Solids, g/L | 109 | | 112 | | 118 | | - | |

| | | | | | | | | |
|---|---|---|---|---|---|---|---|---|
| * includes fill time, heating time to 120°C and time at 120°C after warm fill. | | | | | | | | |

**TABLE 3B**

| *PULPING STUDY SUMMARY* | | | | | | |
|---|---|---|---|---|---|---|
| COOK NUMBER | | | | | | |
| *BEST COOK: NEW RDH COOKING PROCEDURE* | | | | | R3 | R4 |
| | | | | | | |
| *BASELINE COOK: OLD RDH COOKING PROCEDURE* | | | | | R7 | R8 |
| | | | | | | |
| *BEST DO-ABLE COOK*: *MODIFIED NEW RDH COOKING PROCEDURE* | | | | | R12 | |

| COOKING CONDITIONS | | | | | | |
|---|---|---|---|---|---|---|
| | R3 | R4 | R7 | R8 | R12 | |
| WARM FILL | | | | | | |
| EA (g/l) as Na20 | 18 | 18.6 | 18 | 18.6 | 17.7 | |
| Solids, % | 14.3 | 14.1 | 14.7 | 14.6 | 15 | |
| HOT FILL | | | | | | |
| EA (g/l) Na20 % | 20 | 19.8 | 18 | 18.3 | 19.6 | |
| Solids, | 11.9 | 12.7 | 17 | 17 | 17.3 | |
| COOKING STAGE | | | | | | |
| AA Charge, % | 16 | 16 | 10 | 10 | 16 | |
| H-FACTOR | 475 | 452 | 831 | 832 | 494 | |
| MAXIMUM TEMP. DEGREE C | 160 | 160 | 170 | 170 | 160 | |
| DISPLACEMENT | | | | | | |
| EA (g/l) as Na20 | 9 | 10.1 | 3.7 | 3.5 | 10.7 | |
| Solids, % | 0 | 0 | 10.4 | 10.3 | 10 | |

### EXAMPLE 1

The following definitive pulps were produced for the bleaching study:

| Case | Cook No. | Kappa | Brightness, TAPPI |
|---|---|---|---|
| "Best" | R3 | 8.8 | 45.3 |
| | R4 | 9.3 | 45.0 |
| "Baseline" | R7 | 8.9 | 40.6 |
| | R8 | 8.8 | 41.3 |
| "Best Do-able" | R10 | 8.5 | 41.5 |
| | R11 | 9.2 | 40.8 |
| | R12 | 9.3 | 41.5 |

Five RDH pulps (R3, R4, R7, R8 and R12) were bleached using an (O)(D100)(EO)(D) sequence. However, each of the five RDH pulps were first oxygen delignified in stirred reactors using the conditions shown below in Table 4.

**TABLE 4**

| OXYGEN DELIGNIFICATION CONDITIONS | | | | | |
|---|---|---|---|---|---|
| | Best Case | | Baseline Case | | "Do-able " Best Case |
| Sample identification | R3 | R4 | R7 | R8 | R12 |
| Species | Aspen | Aspen | Aspen | Aspen | Aspen |
| Cook type | RDH | RDH | RDH | RDH | RDH |
| Kappa | 8.8 | 9.2 | 8.9 | 8.8 | 9.3 |
| Viscosity, mPa.s | 40.7 | 44.9 | 33.3 | 32.2 | 32.1 |
| Unbl. brightness, % | 45.3 | 45 | 40.6 | 41.3 | 41.5 |
| | | | | | |
| | | | | | |
| | | | | | |
| | | | | | |

| O-Stage: 6.78 bar (95 psig), 99°C. 12% cons. | | | | | |
|---|---|---|---|---|---|
| NaOH, % | 2 | 2 | 2 | 2 | 2 |
| O2 time, min | 60 | 60 | 60 | 60 | 60 |
| Final pH | 12.8 | 12.9 | 12.5 | 12.5 | 12.3 |
| Kappa | 4.7 | 5.2 | 4.7 | 4.5 | 5 |
| Viscosity, mPa.s | 14.4 | 13.8 | 12.6 | 13.6 | 12.5 |
| Kappa reduction, % | 46.6 | 43.5 | 47.2 | 48.9 | 50 |
| Yield on raw stock, % | 95.2 | 95.8 | 94.3 | 98.8 | 94.4 |

For the bleaching studies, a 0.225 kappa factor was used in calculating the chlorine dioxide charge in the D100-stage for pulps R3, R7 and R12. A 0.27 kappa factor was used for pulps R4, R8 and R12. Tables 5 through 10 below show the (D100) (Eo)(D) bleaching conditions and results on the oxygen delignified pulps from these cooks. The chlorine dioxide solution concentration was adjusted by a 0.92 factor to compensate for losses of chlorine dioxide in charging the reactors and polyethylene bags during bleaching.

**TABLE 5**

| Bleaching with (O)(D100)(Eo)D on Optimal RDH Pulp | | | | | | | | |
|---|---|---|---|---|---|---|---|---|
| **Kappa factor = 0.225** | | | | | | | | |

| Sample identification | | | R3 | | | | | |
|---|---|---|---|---|---|---|---|---|
| Species | | | Aspen | | | | | |
| Cook type | | | RDH | | | | | |
| 02 Pulp Kappa | | | 4.7 | | | | | |
| Viscosity, mPa.s | | | 14.4 | | | | | |

| **D-100-Stage: 30 min. 68°C. 4.2% cons.** | | | | | | | | |
|---|---|---|---|---|---|---|---|---|
| Chlorination factor | | | 0.23 | | | | | |
| ClO2, % as available Cl₂* | | | 1.06 | | | | | |
| Actual ClO2, % as avail. Cl₂ | | | 1.15 | | | | | |
| Substitution, % | | | 100 | | | | | |
| H2SO4, % | | | 1.5 | | | | | |
| Final pH | | | 2 | | | | | |
| Residual, g/L avail. Cl₂ | | | 0.14 | | | | | |

| **EO-Stage: 60 min. 74°C. 10% cons.** | | | | | | | | |
|---|---|---|---|---|---|---|---|---|
| NaOH, % | | | 0.8 | | | | | |
| 02 pressure, psig | | | 25 | | | | | |
| 02 time, minutes | | | 15 | | | | | |
| Final pH | | | 12.4 | | | | | |
| K No. (25 Ml) | | | 2.3 | | | | | |
| Viscosity, mPa.s | | | 13.7 | | | | | |
| Yield on raw stock, % | | | 93.5 | | | | | |

| **D-Stage: 74°C. 210 min. 10% cons.** | | | | | | | | |
|---|---|---|---|---|---|---|---|---|
| Sample number | #1 | #2 | #3 | #4 | #5 | #6 | #7 | #8 |
| C1O2 as C1O2, %* | 0.1 | 0.3 | 0.5 | 0.7 | 0.9 | 1.1 | 0.9 | 1.1 |
| Actual ClO2, % ClO2 | 0.11 | 0.33 | 0.54 | 0.76 | 0.98 | 1.2 | 0.98 | 1.2 |
| NaOH, % | 0 | 0 | 0.09 | 0.16 | 0.25 | 0.3 | 0.33 | 0.42 |
| H2SO4, % | 0.1 | 0.05 | 0 | 0 | 0 | 0 | 0 | 0 |
| Final pH | 4.1 | 3.4 | 3.3 | 3 | 2.9 | 2.6 | 3.6 | 3.7 |
| Residual as C102, % | 0.02 | 0.01 | 0.01 | 0.02 | 0.02 | 0.02 | 0 | 0 |
| Brightness, %ISO | 89.7 | 90.4 | 91.2 | 91.5 | 91.6 | 92 | 91.1 | 91.3 |
| Viscosity, mPa.s | 13.1 | - | - | 11.2 | - | - | - | 9.2 |

| | | | | | | | | |
|---|---|---|---|---|---|---|---|---|
| * Actual ClO2 concentration x 0.92 | | | | | | | | |

**TABLE 6**

| Bleaching with (O)(D100)(Eo)(D) on Optimal RDH Pulp | | | | | | | | |
|---|---|---|---|---|---|---|---|---|
| Kappa factor = 0.27 | | | | | | | | |
| Sample identification | | | R4 | | | | | |
| Species | | | Aspen | | | | | |
| Cook type | | | RDH | | | | | |
| 02 Pulp Kappa | | | 5.2 | | | | | |
| Viscosity, mPa.s | | | 13.8 | | | | | |

| D-100-Stage: 30 min. 68°C. 4.2% cons. | | | | | | | | |
|---|---|---|---|---|---|---|---|---|
| Chlorination factor | | | 0.27 | | | | | |
| ClO2, % as available Cl₂* | | | 1.4 | | | | | |
| Actual ClO2, as avail. Cl₂ | | | 1.53 | | | | | |
| Substitution, % | | | 100 | | | | | |
| H2SO4, % | | | 2 | | | | | |
| Final pH | | | 1.9 | | | | | |
| Residual, g/L avail. Cl₂ | | | 0.09 | | | | | |

| **EO-Stage: 60 min. 74°C. 10% cons.** | | | | | | | | |
|---|---|---|---|---|---|---|---|---|
| NaOH, % | | | 0.8 | | | | | |
| O2 pressure, psig | | | 25 | | | | | |
| O2 time, minutes | | | 15 | | | | | |
| Final pH | | | 12.5 | | | | | |
| K No. (25 Ml) | | | 2 | | | | | |
| Viscosity, mPa.s | | | 13.3 | | | | | |
| Yield on raw stock, % | | | 92.8 | | | | | |

| **D-Stage: 74°C. 210 min. 10% cons.** | | | | | | | | |
|---|---|---|---|---|---|---|---|---|
| Sample number | #1 | #2 | #3 | #4 | #5 | #6 | #7 | #8 |
| ClO2 as ClO2, %* | 0.1 | 0.3 | 0.5 | 0.7 | 0.9 | 1.1 | 0.9 | 1.1 |
| Actual ClO2, % ClO2 | 0.11 | 0.33 | 0.54 | 0.76 | 0.98 | 1.2 | 0.98 | 1.2 |
| NaOH, % | 0 | 0 | 0.09 | 0.16 | 0.25 | 0.3 | 0.33 | 0.42 |
| H2SO4, % | 0.1 | 0.05 | 0 | 0 | 0 | 0 | 0 | 0 |
| Final pH | 4.3 | 3.4 | 3.4 | 3.2 | 2.8 | 2.7 | 3.7 | 3.5 |
| Residual as ClO2, % | 0.01 | 0.01 | 0.01 | 0.02 | 0.01 | 0.01 | 0 | |
| Brightness, %ISO | 89.8 | 90.5 | 91.2 | 91.5 | 91.8 | 91.8 | 91.4 | 91.5 |
| Viscosity, mPa.s | 12.5 | - | - | 11.6 | - | - | - | 9.8 |

| | | | | | | | | |
|---|---|---|---|---|---|---|---|---|
| * Actual ClO2 concentration x 0.92 | | | | | | | | |

**TABLE 7**

| **Bleaching with (O)(D100)(Eo)(D) on Baseline RDH Pulp** | | | | | | |
|---|---|---|---|---|---|---|
| Kappa factor = 0.225 | | | | | | |
| Sample identification | | | R7 | | | |
| Species | | | Aspen | | | |
| Cook type | | | RDH | | | |
| 02 Pulp Kappa | | | 4.5 | | | |
| Viscosity, mPa.s | | | 13.6 | | | |

| **(D100)-Stage: 30 min. 68°C. 4.2% cons.** | | | | | | |
|---|---|---|---|---|---|---|
| Chlorination factor | | | 0.23 | | | |
| ClO2, % as available Cl₂* | | | 1.01 | | | |
| Actual ClO2, % as avail. C12 | | | 1.1 | | | |
| Substitution, % | | | 100 | | | |
| H2SO4, % | | | 2 | | | |
| Final pH | | | 2.7 | | | |
| Residual, g/L avail. C12 | | | 0.01 | | | |

| **EO-Stage: 60 min. 74°C. 10% cons.** | | | | | | |
|---|---|---|---|---|---|---|
| NaOH, % | | | 0.8 | | | |
| O2 pressure, psig | | | 25 | | | |
| O2 time, minutes | | | 15 | | | |
| Final pH | | | 12.3 | | | |
| K No. (25 Ml) | | | 2.3 | | | |
| Viscosity, mPa.s | | | 13.3 | | | |
| Yield on raw stock, % | | | 97 | | | |

| **D-Stage: 74°C. 210 min. 10% cons.** | | | | | | |
|---|---|---|---|---|---|---|
| Sample number | #1 | #2 | #3 | #4 | #5 | #6 |
| ClO2 as ClO2, %* | 0.1 | 0.3 | 0.5 | 0.7 | 0.9 | 1.1 |
| Actual ClO2, % ClO2 | 0.11 | 0.33 | 0.54 | 0.76 | 0.98 | 1.2 |
| NaOH, % | 0 | 0 | 0.08 | 0.2 | 0.33 | 0.42 |
| H2SO4, % | 0.1 | 0.05 | 0 | 0 | 0 | 0 |
| Final pH | 4 | 3.5 | 3.4 | 3.4 | 3.4 | 3.8 |
| Residual as ClO2, % | 0 | 0 | 0 | 0 | 0 | 0 |
| Brightness, %ISO | 87.6 | 88.7 | 89.7 | 90.3 | 90.3 | 90.6 |
| Viscosity, mPa.s | 12.6 | - | - | 11.4 | - | 9.6 |

| | | | | | | |
|---|---|---|---|---|---|---|
| * Actual ClO2 concentration x 0.92 | | | | | | |

**TABLE 8**

| **Bleaching with (O)(D100)(Eo)(D) on Baseline RDH Pulp** | | | | | | |
|---|---|---|---|---|---|---|
| Kappa factor = 0.27 | | | | | | |
| Sample identification | | | R8 | | | |
| Species | | | Aspen | | | |
| Cook type | | | RDH | | | |
| O2 Pulp Kappa | | | 4.7 | | | |
| Viscosity, mPa.s | | | 12.6 | | | |

| **(D100)-Stage: 30 min. 68°C. 4.2% cons.** | | | | | | |
|---|---|---|---|---|---|---|
| Chlorination factor | | | 0.27 | | | |
| ClO2, % as available Cl₂* | | | 1.27 | | | |
| Actual ClO2, as avail. Cl₂ | | | 1.38 | | | |
| Substitution, % | | | 100 | | | |
| H2SO4, % | | | 2 | | | |
| Final pH | | | 1.9 | | | |
| Residual, g/L avail. C12 | | | 0.07 | | | |

| **EO-Stage: 60 min. 74°C. 10% cons.** | | | | | | |
|---|---|---|---|---|---|---|
| NaOH, % | | | 0.8 | | | |
| O2 pressure, psig | | | 25 | | | |
| O2 time, minutes | | | 15 | | | |
| Final pH | | | 12.2 | | | |
| K No. (25 Ml) | | | 2.1 | | | |
| Viscosity, mPa.s | | | 12.6 | | | |
| Yield on raw stock, % | | | 94.2 | | | |

| **D-Stage: 74°C. 210 min. 10% cons.** | | | | | | |
|---|---|---|---|---|---|---|
| Sample number | #1 | #2 | #3 | #4 | #5 | #6 |
| ClO2 as ClO2, %* | 0.1 | 0.3 | 0.5 | 0.7 | 0.9 | 1.1 |
| Actual ClO2, % ClO2 | 0.11 | 0.33 | 0.54 | 0.76 | 0.98 | 1.2 |
| NaOH, % | 0 | 0 | 0.08 | 0.2 | 0.33 | 0.42 |
| H2SO4, % | 0.1 | 0.05 | 0 | 0 | 0 | 0 |
| Final pH | 3.6 | 3.1 | 3.1 | 3.1 | 3.2 | 3.6 |
| Residual as ClO2, % | 0 | 0 | 0 | 0 | 0 | 0 |
| Brightness, %ISO | 87 | 88.7 | 89:3 | 90.1 | 90.5 | 90.5 |
| Viscosity, mPa.s | 12.2 | - | - | 11.2 | - | 9.5 |

| | | | | | | |
|---|---|---|---|---|---|---|
| * Actual ClO2 concentration x 0.92) | | | | | | |

**TABLE 9**

| **Bleaching with (O)(D100)(Eo)(D) on Best"Do-able" RDH Pulp** | | | | | | |
|---|---|---|---|---|---|---|
| **Kappa factor = 0.225** | | | | | | |
| Sample identification | | | R12 | | | |
| Species | | | Aspen | | | |
| Cook type | | | RDH | | | |
| O2 Pulp Kappa | | | 5 | | | |
| Viscosity, mPa.s | | | 12.5 | | | |

| **D-100-Stage: 30 min. 68°C. 4.2% cons.** | | | | | | |
|---|---|---|---|---|---|---|
| Chlorination factor | | | 0.03 | | | |
| ClO2, % as available Cl₂* | | | 1.13 | | | |
| Actual ClO2, % as avail. Cl₂ | | | 1.22 | | | |
| Substitution, % | | | 100 | | | |
| H2SO4, % | | | 1.5 | | | |
| Final pH | | | 2 | | | |
| Residual, g/L avail. Cl₂ | | | 0.04 | | | |

| **EO-Stage: 60 min. 74°C. 10% cons.** | | | | | | |
|---|---|---|---|---|---|---|
| NaOH, % | | | 0.8 | | | |
| O2 pressure, psig | | | 25 | | | |
| O2 time, minutes | | | 15 | | | |
| Final pH | | | 12.7 | | | |
| K No. (25 Ml) | | | 2.3 | | | |
| Viscosity, mPa.s | | | 11.9 | | | |
| Yield on raw stock, % | | | - | | | |

| **D-Stage: 74°C. 210 min. 10% cons.** | | | | | | |
|---|---|---|---|---|---|---|
| Sample number | #1 | #2 | #3 | #4 | #5 | #6 |
| ClO2 as ClO2, % | 0.1 | 0.3 | 0.5 | 0.7 | 0.9 | 1.1 |
| Actual ClO2, % ClO2 | 0.11 | 0.33 | 0.54 | 0.76 | 0.98 | 1.2 |
| NaOH, % | 0 | 0 | 0.08 | 0.2 | 0.33 | 0.42 |
| H2SO4, % | 0.1 | 0.05 | 0 | 0 | 0 | 0 |
| Final pH | 4.1 | 3.7 | 3.4 | 3.4 | 3.4 | 3.3 |
| Residual as ClO2, % | 0.01 | 0.01 | 0.01 | 0.01 | 0.01 | 0.01 |
| Brightness, %ISO | 88.9 | 90 | 90.8 | 91 | 91.6 | 91.8 |
| Viscosity, mPa.s | 11.9 | - | - | 10.5 | - | 9.4 |

| | | | | | | |
|---|---|---|---|---|---|---|
| * Actual ClO2 concentration x 0.92 | | | | | | |

**TABLE 10**

| **Bleaching with (O)(D100)(Eo)(D) on Best "Do-able" RDH Pulp** | | | | | | |
|---|---|---|---|---|---|---|
| **Kappa factor = 0.27** | | | | | | |
| Sample identification | | | R12 | | | |
| Species | | | Aspen | | | |
| Cook type | | | RDH | | | |
| 02 Pulp Kappa | | | 5 | | | |
| Viscosity, mPa.s | | | 12.5 | | | |

| **D-100-Stage: 30 min. 68°C. 4.2% cons.** | | | | | | |
|---|---|---|---|---|---|---|
| Chlorination factor | | | 0.03 | | | |
| ClO2, % as available Cl₂* | | | 1.35 | | | |
| Actual ClO2, % as avail. Cl₂ | | | 1.47 | | | |
| substitution, % | | | 100 | | | |
| H2SO4, % | | | 2 | | | |
| Final pH | | | 2.3 | | | |
| Residual, g/L avail. Cl₂ | | | 0.08 | | | |

| **EO-Stage: 60 min. 74°C. 10% cons.** | | | | | | |
|---|---|---|---|---|---|---|
| NaOH, % | | | 0.8 | | | |
| O2 pressure, psig | | | 25 | | | |
| O2 time, minutes | | | 15 | | | |
| Final pH | | | 12.6 | | | |
| K No. (25 Ml) | | | 2.2 | | | |
| Viscosity, mPa.s | | | 12.2 | | | |
| Yield on raw stock, % | | | - | | | |

| **D-Stage: 74°C. 210 min. 10% cons.** | | | | | | |
|---|---|---|---|---|---|---|
| Sample number | #1 | #2 | #3 | #4 | #5 | #6 |
| ClO2 as ClO2, %* | 0.1 | 0.3 | 0.5 | 0.7 | 0.9 | 1.1 |
| Actual ClO2, % ClO2 | 0.11 | 0.33 | 0.54 | 0.76 | 0.98 | 1.2 |
| NaOH, % | 0 | 0 | 0.08 | 0.2 | 0.33 | 0.42 |
| H2SO4, % | 0.1 | 0.05 | 0 | 0 | 0 | 0 |
| Final pH | 3.9 | 3.4 | 3.3 | 3.3 | 3.3 | 3.2 |
| Residual as ClO2, | 0.01 | 0.01 | 0.01 | 0.01 | 0 | 0.01 |
| Brightness, %ISO | 88.9 | 90 | 90.8 | 91.1 | 91.5 | 91.8 |
| Viscosity, mPa.s | 12.4 | - | - | 10.7 | - | 9.5 |

| | | | | | | |
|---|---|---|---|---|---|---|
| * Actual ClO2 concentration x 0.92 | | | | | | |

As shown in FIGS. 5 and 5A, the use of a higher kappa factor did not appear to reduce the D1-stage chlorine dioxide requirements. The best case RDH pulps (R3 and R4) produced 1.5 to 2 points higher brightness than the baseline case RDH pulps (R7 and R8) at equivalent chlorine dioxide charges.

From FIGS. 6 and 6A, it is shown that the best do-able case RDH pulp (R12) produced intermediate brightness between the best case RDH pulp (R3) and the baseline case RDH pulp (R7).

FIGS. 7 and 7A show that the best do-able case RDH pulp (R12) gave intermediate brightness between the best case RDH pulp (R4) and the baseline case RDH pulp (R8).

From the pulp bleaching studies, a summary of the results is shown below in Table 11. The easiest pulps to bleach were the best case pulps. The most difficult to bleach were the baseline case pulps with the bleachability of the best do-able case falling between the first two cases. Results indicated that a combination of high alkalinity (white liquor addition at the warm and hot fill mode plus cooking stage, AA charge between 15% AA and 35% AA) and a low cooking temperature (approximately 150°C ∼ 167°C) improves pulp bleachability and, thus, final brightness of pulp. It should be noted that the black liquor strength during the RDH cook should be maintained.

## Claims

1. A batch digesting process of the type using rapid displacement heating to produce delignified pulp, wherein spent liquor produced in a digester (10) as a result of cooking a mass of cellulosic material with cooking liquor is displaced and collected in accumulators (24,28,58) as hot black liquor and as warm black liquor so as to conserve and utilize the heat of the spent liquor to preheat another mass of cellulosic material in warm black liquor and hot black liquor displacement type pretreatments with progressively hotter spent liquors prior to cooking, wherein:
white liquor is added to the warm black liquor during the warm black liquor pretreatment and to the hot black liquor during the hot black liquor pretreatment stages and to the cooking liquor during the cooking stage in the digesting process, the total white liquor added having a distributed charge between approximately 15% active alkalinity and about 35% active alkalinity; and
the temperature of the cooking liquor is raised to between 150° ∼ 167°C for the cooking stage.

2. The process of Claim 1, wherein the white liquor solution is added to the warm black liquor (temperature between 90° and 150°C) and to the hot black liquor (temperature between 150° and 167°C) in a predetermined amount.

3. The process of Claim 1, wherein white liquor is added to a cool black liquor (temperature between 70° and 90°C), and the mass of cellulosic material is pretreated with said cool black liquor with white liquor added thereto, before the warm black liquor pretreatment.

4. The process of Claim 1, wherein the preferred total white liquor charge is > 20% AA.

5. The process of Claim 1, wherein the preferred cooking temperature ranges between 155° ∼ 167°C.

6. A method for producing bleachable grade pulp according to the process of Claim 1, comprising the steps of:
(a) introducing wood chips into the digester (10);
(b) pretreating the chips with a mixture of warm black liquor and white liquor below cooking temperature;
(c) displacing the mixture from the digester (10) with at least one mixture of a hot black liquor and hot white liquor;
(d) increasing the temperature of the digester (10) to the cooking temperature;
(e) maintaining said temperature until the chips are digested;
(f) displacing the contents of the digester (10) with a liquid filtrate derived from pulp washing; and
(g) emptying the contents of the digester (10) by applying gas pressure to the interior of the digester (10) or pumping out.

7. The method of Claim 6, including the step of pretreating the chips with a mixture of cool black liquor and white liquor (or NaOH solution), before the step of pretreating with warm black liquor.

8. The method of Claim 6, wherein the total white liquor used has a total charge ranging between 15% AA ∼ 35% AA.

9. The method of Claim 6, including the step of displacing the contents of the digester (10) with any combination of washer filtrate and white liquor (or NaOH solution).

## Patentansprüche

1. Verfahren zum chargenweisen Aufschließen des Typs, bei dem eine Schnellverdrängungserhitzung verwendet wird, um entlignifizierten Zellstoff herzustellen, wobei verbrauchte Lauge, die in einem Kocher (10) infolge des Kochens einer Masse von Cellulosematerial mit Kochlauge erzeugt wird, verdrängt und in Akkumulatoren (24, 28, 58) als heiße Schwarzlauge und als warme Schwarzlauge gesammelt wird, um so die Wärme der verbrauchten Lauge zu konservieren und auszunutzen, um eine weitere Masse von Cellulosematerial in Warmschwarzlaugen- und Heißschwarzlaugenverdrängungsvorbehandlungen mit fortschreitend heißeren verbrauchten Laugen vor dem Kochen vorzubehandeln, wobei:
Weißlauge der warmen Schwarz lauge während der Warmschwarzlaugenvorbehandlungsstufe und der heißen Schwarz lauge während der Heißschwarzlaugenvorbehandlungsstufe und der Kochlauge während der Kochstufe in dem Aufschlußprozeß zugesetzt wird, wobei die gesamte zugesetzte Weißlauge einen verteilten Eintrag zwischen etwa 15% aktiver Alkalinität und etwa 35% aktiver Alkalinität hat; und
die Temperatur der Kochlauge auf einen Wert zwischen 150 °C ∼ 167 °C für die Kochstufe erhöht wird.

2. Verfahren nach Anspruch 1, wobei die Weißlaugenlösung der warmen Schwarzlauge (Temperatur zwischen 90 °C und 150 °C) und der heißen Schwarzlauge (Temperatur zwischen 150 °C und 167 °C) in einer vorbestimmten Menge zugesetzt wird.

3. Verfahren nach Anspruch 1, wobei Weißlauge einer kalten Schwarzlauge (Temperatur zwischen 70 °C und 90 °C) zugesetzt wird und die Masse von Cellulosematerial mit der kalten Schwarzlauge mit dieser zugesetzter Weißlauge vor der Vorbehandlung mit warmer Schwarz lauge vorbehandelt wird.

4. Verfahren nach Anspruch 1, wobei der bevorzugte gesamte Weißlaugeneintrag > 20% AA ist.

5. Verfahren nach Anspruch 1, wobei die bevorzugte Kochtemperatur in einem Bereich zwischen 155 °C ∼ 167 °C liegt.

6. Verfahren zum Herstellen von Zellstoff von bleichbarer Qualität gemäß dem Verfahren nach Anspruch 1, beinhaltend die Schritte:
(a) Einbringen von Holzschnitzeln in den Kocher (10);
(b) Vorbehandeln der Schnitzel mit einer Mischung aus warmer Schwarz lauge und Weißlauge unterhalb der Kochtemperatur;
(c) Verdrängen der Mischung aus dem Kocher (10) mit wenigstens einer Mischung aus einer heißen Schwarz lauge und einer heißen Weißlauge;
(d) Erhöhen der Temperatur des Kochers (10) auf die Kochtemperatur;
(e) Aufrechterhalten dieser Temperatur, bis die Schnitzel aufgeschlossen sind;
(f) Verdrängen des Inhalts des Kochers (10) mit einem flüssigen Filtrat, das aus der Zellstoffwaschung gewonnen wird; und
(g) Entleeren des Inhalts des Kochers (10) durch Beaufschlagen des Inneren des Kochers (10) mit Gasdruck oder durch Abpumpen.

7. Verfahren nach Anspruch 6, beinhaltend den Schritt Vorbehandeln der Schnitzel mit einer Mischung aus kalter Schwarz lauge und Weißlauge (oder NaOH-Lösung) vor dem Schritt des Vorbehandelns mit warmer Schwarzlauge.

8. Verfahren nach Anspruch 6, wobei die gesamte verwendete Weißlauge einen Gesamteintrag hat, der in einem Bereich zwischen 15% AA ∼ 35% AA liegt.

9. Verfahren nach Anspruch 6, beinhaltend den Schritt Verdrängen des Inhalts des Kochers (10) mit irgendeiner Kombination aus Wascherfiltrat und Weißlauge (oder NaOH-Lösung).

## Revendications

1. Procédé de lessivage par lots du type utilisant un chauffage à déplacement rapide pour produire de la pâte délignifiée, dans lequel on déplace la liqueur consommée produite dans un lessiveur (10) suite à la cuisson d'une masse de matière cellulosique avec de la liqueur de cuisson, et on la récolte dans des accumulateurs (24, 28, 58) sous forme de liqueur noire très chaude et sous forme de liqueur noire chaude de façon à conserver et à utiliser la chaleur de la liqueur consommée pour préchauffer une autre masse de matière cellulosique dans des prétraitements du type à déplacement de liqueur noire chaude et de liqueur noire très chaude, avec des liqueurs consommées de plus en plus chaudes, avant de procéder à la cuisson, dans lequel:
on ajoute de la liqueur blanche à la liqueur noire chaude au cours de l'étape de prétraitement faisant appel à de la liqueur noire chaude et à la liqueur noire très chaude au cours de l'étape de prétraitement faisant appel à de la liqueur noire très chaude, ainsi qu'à la liqueur de cuisson au cours de l'étape de cuisson dans le procédé de lessivage, la liqueur blanche totale ajoutée possédant une charge distribuée s'étendant entre une alcalinité active à concurrence d'approximativement 15% et une alcalinité active à concurrence d'environ 35%; et
on élève la température de la liqueur de cuisson à une valeur entre 150° ∼ 167°c pour l'étape de cuisson.

2. Procédé selon la revendication 1, dans lequel on ajoute la solution de liqueur blanche à la liqueur noire chaude (température entre 90°C et 150°C) et à la liqueur noire très chaude (température entre 150° et 167°C) en une quantité prédéterminée.

3. Procédé selon la revendication 1, dans lequel on ajoute de la liqueur blanche à une liqueur noire froide (température entre 70° et 90°C) et on soumet la masse de matière cellulosique à un prétraitement avec ladite liqueur noire froide à laquelle on a ajouté de la liqueur blanche, avant de procéder au prétraitement faisant appel à de la liqueur noire chaude.

4. Procédé selon la revendication 1, dans lequel la charge de liqueur blanche totale préférée représente une valeur AA >20%.

5. Procédé selon la revendication 1, dans lequel la température de cuisson préférée se situe dans le domaine de 155° ∼ 167°C.

6. Procédé pour produire de la pâte de qualité apte à être blanchie selon le procédé de la revendication 1, comprenant les étapes consistant à:
(a) introduire des copeaux de bois dans le lessiveur (10);
(b) soumettre les copeaux à un prétraitement avec un mélange de liqueur noire chaude et de liqueur blanche à une température inférieure à la température de cuisson;
(c) déplacer le mélange du lessiveur (10) avec au moins un mélange de liqueur noire très chaude et de liqueur blanche très chaude;
(d) élever la température du lessiveur (10) à la température de cuisson;
(e) maintenir ladite température jusqu'à ce que le lessivage des copeaux soit terminé;
(f) déplacer le contenu du lessiveur (10) avec un filtrat liquide dérivé du lavage de la pâte; et
(g) vider le contenu du lessiveur (10) en appliquant une pression de gaz à l'intérieur du lessiveur (10) ou encore l'évacuer par pompage.

7. Procédé selon la revendication 6, englobant l'étape consistant à prétraiter les copeaux avec un mélange de liqueur noire froide et de liqueur blanche (ou d'une solution de NaOH) avant l'étape de prétraitement avec de la liqueur noire chaude.

8. Procédé selon la revendication 6, dans lequel la liqueur blanche totale utilisée possède une charge totale se situant dans le domaine d'une valeur AA de 15% à une valeur AA de 35%

9. Procédé selon la revendication 6, englobant l'étape consistant à déplacer le contenu du lessiveur (10) avec n'importe quelle combinaison de filtrat du cylindre laveur et de liqueur blanche (ou de solution de NaOH).
